# EUROPEAN PATENT SPECIFICATION

(11) **EP 2 097 566 B1**
(45) Date of publication and mention of the grant of the patent: **21.09.2011**
(21) Application number: 07839398.0
(22) Date of filing: 09.10.2007
(51) Int. Cl.: D02G 3/04, A41D 31/00, A41D 19/015

(54) **CUT RESISTANT FABRIC COMPRISING ARAMID FIBERS OF DIFFERENT DENIER AND METHOD FOR MAKING ARTICLES THEREFROM**
SCHNEIDFESTES TEXTILES FLÄCHENGEBILDE MIT ARAMIDFASERN UNTERSCHIEDLICHER TITER UND VERFAHREN ZUR HERSTELLUNG VON ERZEUGNISSEN DARAUS
TISSUS ET ARTICLES RÉSISTANTS AUX COUPURES EN FIBRES À TITRES MULTIPLES ET LEURS PROCÉDÉS DE FABRICATION

(30) Priority: 10.10.2006 US 545177
(43) Date of publication of application: 09.09.2009
(73) Proprietor: E.I. DU PONT DE NEMOURS AND COMPANY, Wilmington, DE 19898 (US)
(72) Inventor: PRICKETT, Larry, John, Chesterfield, VA 23838 (US)
(74) Representative: Dannenberger, Oliver Andre
(86) International application number: PCT/US2007/021582
(87) International publication number: WO 2008/045441

(56) References cited:
- WO-A-2008/017400
- DE-U1-202004 005 008
- US-A- 4 918 912
- US-B1- 6 254 988

## Description

### BACKGROUND OF THE INVENTION

### 1. Field of the Invention.

This invention relates to cut resistant fabrics and articles including gloves and methods of making the same.

### 2. Description of Related Art.

United States Patent Application Publication US 2004/0235383 to Perry et al. discloses a yarn or fabric useful in protective garments designed for activities where exposure to molten substance splash, radiant heat, or flame is likely to occur. The yarn or fabric is made of flame resistant fibers and micro-denier flame resistant fibers. The weight ratio of the flame resistant fibers to the micro-denier flame resistant fibers is in the range of 4-9:2-6.

United States Patent Application Publication US 2002/0106956 to Howland discloses fabrics formed from intimate blends of high-tenacity fibers and low-tenacity fibers wherein the low-tenacity fibers have a denier per filament substantially below that of the high tenacity fibers.

United States Patent Application Publication US 2004/0025486 to Takiue discloses a reinforcing composite yarn comprising a plurality of continuous filaments and paralleled with at least one substantially non-twisted staple fiber yam comprising a plurality of staple fibers. The staple fibers are preferably selected from nylon 6 staple fibers, nylon 66 staple fibers, meta-aromatic polyamide staple fibers, and para-aromatic polyamide staple fibers.

Articles made from para-aramid fibers have excellent cut performance and command a premium price in the marketplace. Such articles, however, can be stiffer than articles made with traditional textile fibers and in some applications the para-aramid articles can abrade more quickly than desired. Therefore, any improvement in either the comfort, durability or the amount of aramid material needed for adequate cut performance in articles is desired.

US 6,254,988 relates to a cut resistant and abrasion resistant composition composed of cotton, nylon, and p-aramid fibers primarily for use in the sheath for sheath/cor yarns in protective apparel. The use of aramid fibers having different deniers and different colors is not disclosed.

### BRIEF SUMMARY OF THE INVENTION

The present invention relates to a cut resistant fabric, comprising: a yarn comprising an intimate blend of staple fibers, the blend comprising:
a) 20 to 50 parts by weight of a fiber selected from the group of aliphatic polyamide fiber, polyolefin fiber, polyester fiber, acrylic fiber and mixtures thereof; and
b) 50 to 80 parts by weight of an aramid fiber mixture,
based on 100 parts by weight of the fibers of a) and b); wherein the aramid fiber mixture comprises at least a first aramid fiber having a linear density of from 3.7 to 6.7 dtex per filament; and a second aramid fiber having a linear density of from 0.56 to 5.0 dtex per filament; and
wherein the difference in filament linear density of the first aramid fiber to the second aramid fiber is 1.1 dtex per filament or greater.

The present invention further relates to a process for making a cut resistant fabric comprising:
a) blending
   i) 20 to 50 parts by weight of a fiber selected from the group of aliphatic polyamide fiber, polyolefin fiber, polyester fiber, acrylic fiber and mixtures thereof, and
   ii) 50 to 80 parts by weight of an aramid fiber mixture;
      based on 100 parts by weight of the fibers of i) and ii),
      wherein the aramide fiber mixture comprises at least a first aramid fiber having a linear density of from 3.7 to 6.7 dtex per filament; and a second aramid fiber having a linear density of from 0.56 to 5.0 dtex per filament; and
      wherein the difference in filament linear density of the first aramid fiber to the second aramid fiber is 1.1 dtex per filament or greater;
b) forming a spun staple yarn from the blend of fibers; and
c) forming a fabric from the spun staple yarn.

### BRIEF DESCRIPTION OF THE DRAWINGS

Figure 1 is a representation of one possible knitted fabric of this invention.
Figure 2 is one article of this invention in the form of a knitted glove.
Figure 3 is a representation of a section of staple fiber yam comprising one possible intimate blend of fibers.
Figure 4 is an illustration of one possible cross section of a staple yam bundle useful in the fabrics of this invention.
Figure 5 is an illustration of another possible cross section of a staple yam bundle useful in the fabrics of this invention.
Figure 6 is an illustration of the cross section of a prior art staple yarn bundle having commonly used 1.5 denier per filament (1.7 dtex per filament) para-aramid fiber.
Figure 7 is an illustration of a one possible ply yam made from two singles yarns.
Figure 8 is an illustration of one possible cross section of a ply yam made from two different singles yarns.
Figure 9 is an illustration of one possible ply yam made from three singles yarns.

### DETAILED DESCRIPTION OF THE INVENTION

In one embodiment, this invention relates to cut resistant fabric comprising a yam comprising an intimate blend of staple fibers, the blend comprising 20 to 50 parts by weight of a lubricating fiber

selected from the group of aliphatic polyamide fiber, polyolefin fiber, polyester fiber, acrylic fiber, and mixtures thereof; and 50 to 80 parts by weight of an aramid fiber mixture; based on the total weight of the aliphatic polyamide, polyolefin, polyester, and aramid fibers. The aramid fiber mixture comprises at least a first aramid fiber having a linear density of from 3.3 to 6 denier per filament (3.7 to 6.7 dtex per filament); and a second aramid fiber having a linear density of from 0.50 to 4.5 denier per filament (0.56 to 5.0 dtex per filament). In some preferred embodiments the first aramid fiber has a linear density of from 3.3 to 5.0 denier per filament (3.7 to 5.6 dtex per filament) and in some preferred embodiments the second aramid fiber has a linear density of from 1.0 to 4.0 denier per filament (1.1 to 4.4 dtex per filament). The difference in filament linear density of the first aramid fiber to the second aramid fiber is 1 denier per filament (1.1 dtex per filament) or greater. In one preferred embodiment, the aliphatic polyamide fiber, polyolefin fiber, polyester fiber, acrylic fiber, or fiber mixture is present in an amount that is 26 to 40 parts by weight and the aramid fiber mixture is present in an amount that is 60 to 74 parts by weight; based on 100 parts by weight of those fibers. In one most preferred embodiment, the aliphatic polyamide fiber, polyolefin fiber, polyester fiber, acrylic fiber, or fiber mixture and the aramid fiber mixture are present in a weight ratio of about 1:2.

Surprisingly, it has been found that fabrics of this invention have cut resistance equivalent to or greater than a fabric made with commonly used 100% 1.5 denier-per-filament (1.7 dtex per filament) para-aramid fiber yarns. In other words, the cut resistance of a 100% para-aramid fiber fabric can be duplicated by a fabric having at most 80 parts by weight para-aramid fiber. It is believed the three types of fibers, namely the lubricating fiber, higher denier-per-filament aramid fiber, and lower denier-per-filament aramid fiber, work together to provide not only cut resistance but also improved fabric abrasion resistance and flexibility, which translates to improved durability and comfort in use.

The word "fabric" is meant to include any woven, knitted, or non-woven layer structure or the like that utilizes yarns. By "yarn" is meant an assemblage of fibers spun or twisted together to form a continuous strand. As used herein, a yarn generally refers to what is known in the art as a singles yarn, which is the simplest strand of textile material suitable for such operations as weaving and knitting. A spun staple yarn can be formed from staple fibers with more or less twist; a continuous multifilament yarn can be formed with or without twist. When twist is present, it is all in the same direction. As use herein the phrases "ply yarn" and "plied yam" can be used interchangeably and refer to two or more yarns, i.e., singles yarns, twisted or plied together. "Woven" is meant to include any fabric made by weaving; that is, interlacing or interweaving at least two yarns typically at right angles. Generally such fabrics are made by interlacing one set of yams, called warp yarns, with another set of yarns, called weft or fill yarns. The woven fabric can have essentially any weave, such as, plain weave, crowfoot weave, basket weave, satin weave, twill weave, unbalanced weaves, and the like. Plain weave is the most common. "Knitted" is meant to include a structure producible by interlocking a series of loops of one or more yarns by means of needles or wires, such as warp knits (e.g., tricot, milanese, or raschel) and weft knits (e.g., circular or flat). "Non-woven" is meant to include a network of fibers forming a flexible sheet material producible without weaving or knitting and held together by either (i) mechanical interlocking of at least some of the fibers, (ii) fusing at least some parts of some of the fibers, or (iii) bonding at least some of the fibers by use of a binder material. Non-woven fabrics that utilize yarns include primarily unidirectional fabrics, however other structures are possible.

In some preferred embodiments, the fabric of this invention is a knitted fabric, using any appropriate knit pattern and conventional knitting machines. Figure 1 is a representation of a knitted fabric. Cut resistance and comfort are affected by tightness of the knit and that tightness can be adjusted to meet any specific need. A very effective combination of cut resistance and comfort has been found in for example, single jersey knit and terry knit patterns. In some embodiments, fabrics of this invention have a basis weight in the range of 100 to 1000 g/m² (3 to 30 oz/yd²), preferably 170 to 850 g/m² (5 to 25 oz/yd²), the fabrics at the high end of the basis weight range providing more cut protection.

The fabrics of this invention can be utilized in articles to provide cut protection. Useful articles include but are not limited to gloves, aprons, and sleeves. In one preferred embodiment the article is a cut resistant glove that is knitted. Figure 2 is a representation of one such glove **1** having a detail **2** illustrating the knitted construction of the glove.

In the fabrics and articles including gloves of this invention, the difference in filament linear density of the higher denier-per-filament aramid fiber and the lower denier-per-filament aramid fiber is 1 denier per filament (1.1 dtex per filament) or greater. In some preferred embodiments, the difference in filament linear density is 1.5 denier per filament (1.7 dtex per filament) or greater. It is believed the lubricating fiber reduces the friction between fibers in the staple yam bundle, allowing the lower denier-per-filament aramid fiber and the higher denier-per-filament aramid fiber to more easily move in the fabric yarn bundles. Figure 3 is a representation of a section of staple fiber yarn **3** comprising one possible intimate blend of fibers.

Figure 4 is one possible embodiment of a cross-section **A-A'** of the staple fiber yam bundle of Figure 3. The staple fiber yam **4** contains a first aramid fiber **5** having a linear density of from 3.3 to 6 denier per filament (3.7 to 6.7 dtex per filament), and a second aramid fiber **6** having a linear density of from 0.50 to 4.5 denier per filament (0.56 to 5.0 dtex per filament). Lubricating fiber 7 has a linear density in the same range as the second aramid fiber 6. The lubricating fiber is uniformly distributed in the yarn bundle and in many instances acts as to separate the first and second aramid fibers. It is thought this helps avoid substantial interlocking of any aramid fibrils (not shown) that can be present or generated from wear on the surface of aramid fibers and also provides a lubricating effect on the filaments in the yarn bundle, providing fabrics made from such yarns with a more textile fiber character and better aesthetic feel or "hand".

Figure 5 illustrates another possible embodiment of a cross-section **A-A'** of the staple fiber yam bundle of Figure 3. Yarn bundle **11** has the same first and second aramid fibers **5** and **6** as Figure 4 however the lubricating fiber 8 has a linear density of in the same range as the first aramid fiber **5**. In comparison, Figure 6 is an illustration of a cross-section of the yarn bundle of a prior art commonly used 1.5 denier per filament (1.7 dtex per filament) para-aramid staple yarn **12** with 1.5 denier per filament (1.7 dtex per filament) fibers **9**. For simplicity in the figures, in those instances where the lubricating fiber is said to be roughly the same denier as an aramid fiber type, it is shown having the same diameter as that aramid fiber type. The actual fiber diameters may be slightly different due to differences in the polymer densities. While in all of these figures the individual fibers are represented as having a round cross section, and that many of the fibers useful in these bundles preferably can have a round, oval or bean cross-sectional shape, it is understood that fibers having other cross sections can be used in these bundles.

While in the figures these bundles of fibers represent singles yarns, it is understood these multidenier singles yarns can be plied with one or more other singles yarns to make plied yarns. For example, Figure 7 is an illustration of one embodiment of a ply- or plied- yam 14 made from ply-twisting two singles yarns together. Figure 8 is one possible embodiment of a cross-section **B-B'** of the ply yarn bundle of Figure 7 containing two singles yarns, with one singles yarn **15** made from an intimate blend of multidenier staple fibers as described previously and one singles yam **16** made from only one type of filaments. While two different singles are shown in these figures, this is not restrictive and it should be understood the ply yam could contain more than two yarns ply-twisted together. For example, Figure 9 is an illustration of three singles yarns ply-twisted together. It should also be understood the ply yam can be made from two or more singles yarns made from an intimate blend of multidenier staple fibers as described previously, or the ply yam can be made from at least one of the singles yarn made from an intimate blend of multidenier staple fibers and at least one yam having any desired composition, including for example a yarn comprising continuous filament

Surprisingly, the fabric of this invention has improved flexibility over the fabric made with commonly used 1.5 denier per filament (1.7 dtex per filament) fibers, despite the fact the intimate blend utilizes a large number of filaments that have a larger diameter than the diameter of the 1.5 denier per filament (1.7 dtex per filament) fibers.

The cut resistant fabrics such as the gloves of this invention comprise a yam comprising an intimate blend of staple fibers. By intimate blend it is meant the various staple fibers are distributed homogeneously in the staple yam bundle. The staple fibers used in some embodiments of this invention have a length of 2 to 20 centimeters. The staple fibers can be spun into yarns using short-staple or cotton-based yam systems, long-staple or woolen-based yam systems, or stretch-broken yarn systems. In some embodiments the staple fiber cut length is preferably 3.5 to 6 centimeters, especially for staple to be used in cotton based spinning systems. In some other embodiments the staple fiber cut length is preferably 3.5 to 16 centimeters, especially for staple to be used in long staple or woolen based spinning systems. The staple fibers used in many embodiments of this invention have a diameter of 5 to 30 micrometers and a linear density in the range of about 0.5 to 6.5 denier per filament (0.56 to 7.2 dtex per filament), preferably in the range of 1.0 to 5.0 denier per filament (1.1 to 5.6 dtex per filament).

"Lubricating fiber" as used herein is meant to include any fiber that, when used with the multidenier aramid fiber in the proportions designated herein to make a yam, increases the flexibility of fabrics or articles (including gloves) made from that yarn. It is believed that the desired effect provided by the lubricating fiber is associated with the non-fibrillating and yarn-to-yarn frictional properties of the fiber polymer. Therefore, in some preferred embodiments the lubricating fiber is a non-fibrillating or "fibril-free" fiber. In some embodiments the lubricating fiber has a yarn-on-yarn dynamic friction coefficient, when measured on itself, of less than 0:55, and in some embodiments the dynamic friction coefficient is less than 0.40, as measured by the ASTM Method D3412 capstan method at 50 grams load, 170 degree wrap angle, and 30 cm/second relative movement. For example, when measured in this manner, polyester-on-polyester fiber has a measured dynamic friction coefficient of 0.50 and nylon-on-nylon fiber has a measured dynamic friction coefficient of 0.36. It is not necessary that the lubricant fiber have any special surface finish or chemical treatment to provide the lubricating behavior. Depending on the desire aesthetics of the final fabric and article, the lubricating fiber can have a filament linear density equal to filament linear density of one of the aramid fiber types in the yam or can have a filament linear density different from the filament linear densities of the aramid fibers in the yarn.

The lubricating fiber is selected from the group of aliphatic polyamide fiber, polyolefin fiber, polyester fiber, acrylic fiber and mixtures thereof. In some embodiments the lubricating fiber is a thermoplastic fiber. "Thermoplastic" is meant to have its traditional polymer definition; that is, these materials flow in the manner of a viscous liquid when heated and solidify when cooled and do so reversibly time and time again on subsequent heatings and coolings. In some most preferred embodiments the lubricating fiber is a melt-spun or gel-spun thermoplastic fiber.

In some preferred embodiments aliphatic polyamide fiber refers to any type of fiber containing nylon polymer or copolymer. Nylons are long chain synthetic polyamides having recurring amide groups (-NH-CO-) as an integral part of the polymer chain, and two common examples of nylons are nylon 66, which is polyhexamethylenediamine adipamide, and nylon 6, which polycaprolactam. Other nylons can include nylon 11, which is made from 11-amino-undecanoic acid; and nylon 610, which is made from the condensation product of hexamethylenediamine and sebacic acid.

In some embodiments, polyolefin fiber refers to a fiber produced from polypropylene or polyethylene. Polypropylene is made from polymers or copolymers of propylene. One polypropylene fiber is commercially available under the trade name of Marvess® from Phillips Fibers. Polyethylene is made from polymers or copolymers of ethylene with at least 50 mole percent ethylene on the basis of 100 mole percent polymer and can be spun from a melt; however in some preferred embodiments the fibers are spun from a gel. Useful polyethylene fibers can be made from either high molecular weight polyethylene or ultra-high molecular weight polyethylene. High molecular weight polyethylene generally has a weight average molecular weight of greater than 40,000. One high molecular weight melt-spun polyethylene fiber is commercially available from Fibervisions®; polyolefin fiber can also include a bicomponent fiber having various polyethylene and/or polypropylene sheath-core or side-by-side constructions. Commercially available ultra-high molecular weight polyethylene generally has a weight average molecular weight of about one million or greater. One ultra-high molecular weight polyethylene or extended chain polyethylene fiber can be generally prepared as discussed in U.S. Patent No. 4,457,985. This type of gel-spun fiber is commercially available under the trade names of Dyneema® available from Toyobo and Spectra® available from Honeywell.

In some embodiments, polyester fiber refers to any type of synthetic polymer or copolymer composed of at least 85% by weight of an ester of dihydric alcohol and terephthalic acid. The polymer can be produced by the reaction of ethylene glycol and terephthalic acid or its derivatives. In some embodiments the preferred polyester is polyethylene terephthalate (PET). Polyester formulations may include a variety of comonomers, including diethylene glycol, cyclohexanedimethanol, poly(ethylene glycol), glutaric acid, azelaic acid, sebacic acid, isophthalic acid, and the like. In addition to these comonomers, branching agents like trimesic acid, pyromellitic acid, trimethylolpropane and trimethyloloethane, and pentaerythritol may be used. PET may be obtained by known polymerization techniques from either terephthalic acid or its lower alkyl esters (e.g., dimethyl terephthalate) and ethylene glycol or blends or mixtures of these. Useful polyesters can also include polyethylene napthalate (PEN). PEN may be obtained by known polymerization techniques from 2,6 napthalene dicarboxylic acid and ethylene glycol.

In some other embodiments the preferred polyesters are aromatic polyesters that exhibit thermotropic melt behavior. These include liquid crystalline or anisotropic melt polyesters such as available under the tradename of Vectran® available from Celanese. In some other embodiments fully aromatic melt processible liquid crystalline polyester polymers having low melting points are preferred, such as those described in United States Patent No. 5,525,700.

In some embodiments, acrylic fiber refers to a fiber having at least 85 weight percent acrylonitrile units, an acrylonitrile unit being -(CH2-CHCN)-. The acrylic fiber can be made from acrylic polymers having 85 percent by weight or more of acrylonitrile with 15 percent by weight or less of an ethylenic monomer copolymerizable with acrylonitrile and mixtures of two or more of these acrylic polymers. Examples of the ethylenic monomer copolymerizable with acylonitrile include acylic acid, methacrylic acid and esters thereof (methyl acrylate, ethyl acrylate, methyl methacylate, ethyl methacrylate, etc.), vinyl acetate, vinyl chloride, vinylidene chloride, acrylamide, methacylamide, methacrylonitrile, allylsulfonic acid, methanesulfonic acid and styrenesulfonic acid. Acrylic fibers of various types are commercially available from Sterling Fibers, and one illustrative method of making acrylic polymers and fibers is disclosed in U.S. Patent No. 3,047,455.

In some embodiments of this invention, the lubricating staple fibers have a cut index of at least 0.8 and preferably a cut index of 1.2 or greater. In some embodiments the preferred lubricating staple fibers have a cut index of 1.5 or greater. The cut index is the cut performance of a 475 grams/square meter (14 ounces/square yard) fabric woven or knitted from 100% of the fiber to be tested that is then measured by ASTM F1790-97 (measured in grams, also known as the Cut Protection Performance (CPP)) divided by the areal density (in grams per square meter) of the fabric being cut.

In some embodiments of this invention, the preferred aramid staple fibers are para-aramid fibers. By para-aramid fibers is meant fibers made from para-aramid polymers; poly(p-phenylene terephthalamide) (PPD-T) is the preferred para-aramid polymer. By PPD-T is meant the homopolymer resulting from mole-for-mole polymerization of p-phenylene diamine and terephthaloyl chloride and, also, copolymers resulting from incorporation of small amounts of other diamines with the p-phenylene diamine and of small amounts of other diacid chlorides with the terephthaloyl chloride. As a general rule, other diamines and other diacid chlorides can be used in amounts up to as much as about 10 mole percent of the p-phenylene diamine or the terephthaloyl chloride, or perhaps slightly higher, provided only that the other diamines and diacid chlorides have no reactive groups which interfere with the polymerization reaction. PPD-T, also, means copolymers resulting from incorporation of other aromatic diamines and other aromatic diacid chlorides such as, for example, 2,6-naphthaloyl chloride or chloro- or dichloroterephthaloyl chloride; provided, only that the other aromatic diamines and aromatic diacid chlorides be present in amounts which do not adversely affect the properties of the para-aramid.

Additives can be used with the para-aramid in the fibers and it has been found that up to as much as 10 percent, by weight, of other polymeric material can be blended with the aramid or that copolymers can be used having as much as 10 percent of other diamine substituted for the diamine of the aramid or as much as 10 percent of other diacid chloride substituted for the diacid chloride of the aramid.

Para-aramid fibers are generally spun by extrusion of a solution of the para-aramid through a capillary into a coagulating bath. In the case of poly(p-phenylene terephthalamide), the solvent for the solution is generally concentrated sulfuric acid and the extrusion is generally through an air gap into a cold, aqueous, coagulating bath. Such processes are well known and are generally disclosed in U.S. Patent Nos. 3,063,966; 3,767,756; 3,869,429, & 3,869,430. P-aramid fibers are available commercially as Kevlar® brand fibers, which are available from E. I. du Pont de Nemours and Company, and Twaron® brand fibers, which are available from Teijin, Ltd.

This invention also relates to processes for making a cut resistant fabric such as a glove, comprising the steps of blending 20 to 50 parts by weight of a fiber selected from the group of aliphatic polyamide fiber, polyolefin fiber, polyester fiber, acrylic fiber and mixtures thereof, and 50 to 80 parts by weight of an aramid fiber mixture, based on the total weight of the aliphatic polyamide, polyolefin, polyester, and aramid fibers, and wherein the aramid fiber mixture comprises at least a first aramid fiber having a linear density of from 3.3 to 6 denier per filament (3.7 to 6.7 dtex per filament) and a second aramid fiber having a linear density of from 0.50 to 4.5 denier per filament (0.56 to 5.0 dtex per filament), and wherein the difference in filament linear density of the first aramid fiber to the second aramid fiber is 1 denier per filament (1.1 dtex per, filament) or greater; forming a spun staple yarn from the blend of fibers; and forming a fabric from the spun staple yarn. In one preferred embodiment, the aliphatic polyamide fiber, polyolefin fiber, polyester fiber, or fiber mixture is present in an amount that is 26 to 40 parts by weight and the aramid fiber mixture is present in an amount that is 60 to 74 parts by weight; based on 100 parts by weight of those fibers. In one most preferred embodiment, the aliphatic polyamide fiber, polyolefin fiber, polyester fiber acrylic fiber, or fiber mixture and the aramid fiber mixture are present in a weight ratio of about 1:2.

In some preferred embodiments, the intimate staple fiber blend is made by first mixing together staple fibers obtained from opened bales, along with any other staple fibers, if desired for additional functionality. The fiber blend is then formed into a sliver using a carding machine. A carding machine is commonly used in the fiber industry to separate, align, and deliver fibers into a continuous strand of loosely assembled fibers without substantial twist, commonly known as carded sliver. The carded sliver is processed into drawn sliver, typically by, but not limited to, a two-step drawing process.

Spun staple yarns are then formed from the drawn sliver using conventional techniques. These techniques include conventional cotton system, short-staple spinning processes, such as, for example, open-end spinning, ring-spinning, or higher speed air spinning techniques such as Murata air-jet spinning where air is used to twist the staple fibers into a yarn. The formation of spun yarns useful in the fabrics of this invention can also be achieved by use of conventional woolen system, long-staple or stretch-break spinning processes, such as, for example, worsted or semi-worsted ring-spinning. Regardless of the processing system, ring-spinning is the generally preferred method for making cut-resistant staple yarns.

Staple fiber blending prior to carding is one preferred method for making well-mixed, homogeneous, intimate-blended spun yarns used in this invention, however other processes are possible. For example, the intimate fiber blend can be made by cutter blending processes; that is, the various fibers in tow or continuous filament form can be mixed together during or prior to crimping or staple cutting. This method can be useful when aramid staple fiber is obtained from a multidenier spun tow or a continuous multidenier multifilament yarn. For example, a continuous multifilament aramid yam can be spun from solution through a specially-prepared spinneret to create a yarn wherein the individual aramid filaments have two or more different linear densities; the yarn can then be cut into staple to make a multidenier aramid staple blend. A lubricant fiber can be combined with this multidenier aramid blend either by combining the lubricant fiber with the aramid fiber and cutting them together, or by mixing lubricant staple fiber with the aramid staple fiber after cutting. Another method to blend the fibers is by card and/or drawn sliver-blending; that is, to make individual slivers of the various staple fibers in the blend, or combinations of the various staple fibers in the blend, and supplying those individual carded and/or drawn slivers to roving and/or staple yarn spinning devices designed to blend the sliver fibers while spinning the staple yarn. All of these methods are not intended to be limited and other methods of blending staple fibers and making yarns are possible. All of these staple yarns can contain other fibers as long as the desired fabric attributes are not dramatically compromised.

The spun staple yarn of an intimate blend of fibers is then preferably fed to a knitting device to make a knitted glove. Such knitting devices include a range of very fine to standard gauge glove knitting machines, such as the Sheima Seiki glove knitting machine used in the examples that follow. If desired, multiple ends or yarns can be supplied to the knitting machine; that is, a bundle of yarns or a bundle of plied yarns can be co-fed to the knitting machine and knitted into a glove using conventional techniques. In some embodiments it is desirable to add functionality to the gloves by co-feeding one or more other staple or continuous filament yarns with one or more spun staple yam having the intimate blend of fibers. The tightness of the knit can be adjusted to meet any specific need. A very effective combination of cut resistance and comfort has been found in for example, single jersey knit and terry knit patterns.

### TEST METHODS

Cut Resistance. Cut resistance data for the following described fabrics was generated using ASTM 1790-04 "Standard Test Method for Measuring Cut Resistance of Materials Used in Protective Clothing. For this test a Tomodynamometer (TDM -100) test machine was used. In performance of the test, a cutting edge, under specified force, is drawn one time across a sample mounted on a mandrel. The cutting edge is a stainless steel knife blade having a sharp edge 70 millimeters long. The blade supply is calibrated by using a load of 500 g on a neoprene calibration material at the beginning and end of the test. A new cutting edge is used for each cut test. The sample is a rectangular piece of fabric; it is cut 50 x 100 millimeters on the bias at 45 degrees from the warp and fill directions. The mandrel is a rounded electro-conductive bar with a radius of 38 millimeters and the sample along with a narrow copper strip is mounted thereto using double-face tape. The copper strip is sandwiched between the sample and double-face tape. The cutting edge is drawn across the fabric on the mandrel at a right angle with the longitudinal axis of the mandrel. Cut through is recorded when the cutting edge makes electrical contact with the copper strip. At several different forces, the distance drawn from initial contact to cut through is recorded and a graph is constructed of force as a function of distance to cut through. From the graph, the force is determined for cut through at a distance of 0.8 inches or 20 millimeters and is normalized to validate the consistency of the blade supply. The normalized force is reported as the cut resistance force.

### EXAMPLES

In the following examples, fabrics were knitted using staple fiber-based ring-spun yarns. The staple fiber blend compositions were prepared by blending various staple fibers of a type shown in the Table 1 in proportions as shown in Table 2. In all cases the aramid fiber was made from poly(paraphenylene terephthalamide) (PPD-T). This type of fiber is known under the trademark of Kevlar® and was manufactured by E. I. du Pont de Nemours and Company. The lubricant fiber component was semi-dull nylon 66 fiber sold by Invista under the designation Type 420.

**Table 1**

| General | Specific | Linear Density | | Cut Length |
|---|---|---|---|---|
| Fiber Type | Fiber Type | denier / filament | dtex/ filament | centimeters |
| Aramid | PPD-T | 1.5 | 1.7 | 4.8 |
| Aramid | PPD-T | 2.25 | 2.5 | 4.8 |
| Aramid | PPD-T | 4.2 | 4.7 | 4.8 |
| Lubricant | nylon | 1.7 | 1.9 | 3.8 |

The yarns used to make the knitted fabrics were made in the following manner. For the control yam A, approximately seven kilograms of a single type of PPD-T staple fiber was fed directly into a carding machine to make a carded sliver. An equivalent amount (7 to 9 kilograms) of each staple fiber blend composition for yarns 1 through 5 and comparison yarns B through D as shown in Table 2 were then made. The staple fiber blends were made by first hand-mixing the fibers and then feeding the mixture twice through a picker to make uniform fiber blends. Each fiber blend was then fed through a standard carding machine to make carded sliver.

The carded sliver was then drawn using two pass drawing (breaker/finisher drawing) into drawn sliver and processed on a roving frame to make 6560 dtex (0.9 hank count) rovings. Yarns were then produced by ring-spinning two ends of each roving for each composition. 10/1s cotton count yarns were produced having a 3.10 twist multiplier. Each of the final A through D and 1 through 5 yarns were made by plying a pair of the 10/1s yarns together with a balancing reverse twist to make 10/2s yarns.

Each of the 10/2s yarns were knitted into fabric samples using a standard 7 gauge Sheima Seiki glove knitting machine. The machine knitting time was adjusted to produce glove bodies about one meter long to provide adequate fabric samples for subsequent cut testing. Samples were made by feeding 3 ends of 10/2s to the glove knitting machine to yield fabric samples having a basis weight of about 680 g/m² (20 yd²). Standard size gloves were then made having about the same nominal basis weight.

The fabrics were subjected to the aforementioned cut resistance test and the results are shown in Table 2. The table also shows the cut resistance values normalized to an areal density of 680 g/m² (20 oz/yd²).

The cut resistance of the fabrics and gloves made from yarns 1 through 5 were equivalent to the cut resistance of the fabric and glove made from control yarn A on a normalized weight basis. Although the fabric made from yam 2 has a lower cut resistance value than that of the fabric made from control yarn A it is noted that the statistical confidential interval for the cut resistance values can account for the conclusion that these have equivalent cut resistance. The fabrics and gloves made from yarns 1 through 5 also had a subjectively more comfortable "hand" than the fabric and glove made from control yam A.

In addition, comparison fabrics and gloves made from yarns B through D had lower cut resistance than any of the other fabrics or gloves made, which demonstrates how the addition of an aramid fiber having a linear density from 3.3 to 6 denier per filament (3.7 to 6.7 dtex per filament) synergistically acts to increase cut resistance and, in this example, compensate for the lower cut resistance provided by the nylon fiber.

**Table 2**

| Yarn Item | 1.5 dpf Aramid Staple Fiber | 2.25 dpf Aramid Staple Fiber | 4.2 dpf Aramid Staple Fiber | Lubricating Nylon Staple Fiber | Areal density | ASTM 1790-04 Cut Value | Normalized Cut Value |
|---|---|---|---|---|---|---|---|
| Units | weight % | weight % | weight % | weight % | oz/yd² | grams | grams |
| A | 100 | 0 | 0 | 0 | 20.2 | 934 | 926 |
| 1 | 0 | 40 | 40 | 20 | 19.7 | 968 | 983 |
| 2 | 0 | 40 | 20 | 40 | 20.5 | 897 | 875 |
| 3 | 0 | 20 | 40 | 40 | 19.7 | 958 | 973 |
| 4 | 0 | 30 | 30 | 40 | 19.8 | 925 | 934 |
| 5 | 0 | 33.3 | 33.3 | 33.3 | 21.0 | 1032 | 983 |
| B | 0 | 60 | 0 | 40 | 19.8 | 829 | 833 |
| C | 0 | 74 | 0 | 30 | 20.7 | 889 | 859 |
| D | 0 | 80 | 0 | 20 | 21.2 | 913 | 860 |

## Claims

1. A cut resistant fabric, comprising:
a yam comprising an intimate blend of staple fibers, the blend comprising:
a) 20 to 50 parts by weight of a fiber selected from the group of aliphatic polyamide fiber, polyolefin fiber, polyester fiber, acrylic fiber and mixtures thereof; and
b) 50 to 80 parts by weight of an aramid fiber mixture,
based on 100 parts by weight of the fibers of a) and b);
wherein the aramid fiber mixture comprises at least a first aramid fiber (5) having a linear density of from 3.7 to 6.7 dtex per filament; and a second aramid fiber (6) having a linear density of from 0.56 to 5.0 dtex per filament; and
wherein the difference in filament linear density of the first aramid fiber (5) to the second aramid fiber (6) is 1.1 dtex per filament or greater.

2. The cut resistant fabric of claim 1, wherein based on 100 parts by weight of the fibers of a) and b), the fiber of a) is present in an amount that is 26 to 40 parts by weight and the fiber of b) is present in an amount that is 60 to 70 parts by weight.

3. The cut resistant fabric of claim 1, wherein the first or second aramid fiber (5,6) comprises poly(paraphenylene terephthalamide).

4. The cut resistant fabric of claim 1, in the form of a knit.

5. An article comprising the cut resistant fabric of claim 1.

6. The article of claim 5, in the form of a glove:

7. A process for making a cut resistant fabric comprising:
a) blending
i) 20 to 50 parts by weight of a fiber selected from the group of aliphatic polyamide fiber, polyolefin fiber, polyester fiber, acrylic fiber and mixtures thereof, and
ii) 50 to 80 parts by weight of an aramid fiber mixture,
based on 100 parts by weight of the fibers of i) and ii);
wherein the aramid fiber mixture comprises at least a first aramid fiber (5) having a linear density of from 3.7 to 6.7 dtcx per filament; and a second aramid fiber (6) having a linear density of from 0.56 to 5.0 dtex per filament; and
wherein the difference in filament linear density of the first aramid fiber (5) to the second aramid fiber (6) is 1.1 dtex per filament or greater;
b) forming, a spun staple yarn from the blend of fibers; and
c) forming a fabric from the spun staple yarn.

8. The process oaf claim 7, wherein the blending is accomplished at least in part by mixing the fibers of i) and ii) together and carding the fibers to form a sliver containing an intimate staple fiber blend.

9. The process of claim 7, wherein the spun staple yarn is formed using ring spinning.

10. The process of claim 7, wherein the first or second aramid fiber (5,6) comprises poly(paraphenylene terephthalamide).

11. The process of claim 7, wherein the fabric is formed by knitting.

12. The process of claim 11, wherein the knitting is accomplished by co-feeding to a knitting machine a bundle of yarns or plied yarns comprising the spun staple yam from the blend of fibers and one or more other staple fiber yarns or continuous filament yarns.

13. The process of claim 7, wherein the fabric is in the form of a glove.

## Patentansprüche

1. Schnittfester Stoff, umfassend:
ein Garn, das ein inniges Gemisch von Stapelfasern umfasst, wobei die Mischung Folgendes umfasst:
a) 20 bis 50 Gewichtsteile einer Faser, ausgewählt aus der Gruppe der aliphatischen Polyamidfaser, der Polyolefinfaser, der Polyesterfaser, der Acrylfaser und Mischungen davon; und
b) 50 bis 80 Gewichtsteile einer Aramidfasermischung,
basierend auf 100 Gewichtsteilen der Fasern von a) und b);
wobei die Aramidfasermischung mindestens eine erste Aramidfaser (5) mit einer linearen Dichte von 3,7 bis 6,7 dtex pro Filament und eine zweite Aramidfaser (6) mit einer linearen Dichte von 0,56 bis 5,0 dtex pro Filament umfasst; und
wobei der Unterschied in der linearen Dichte der Filamente zwischen der ersten Aramidfaser (5) und der zweiten Aramidfaser (6) 1,1 dtex pro Filament oder mehr beträgt.

2. Schnittfester Stoff nach Anspruch 1, wobei die Faser von a) in einer Menge anwesend ist, die 26 bis 40 Gewichtsteile beträgt und die Faser von b) in einer Menge anwesend ist, die 60 bis 70 Gewichtsteile beträgt, basierend auf 100 Gewichtsteilen der Fasern von a) und b).

3. Schnittfester Stoff nach Anspruch 1, wobei die erste und zweite Aramidfaser (5, 6) Poly(paraphenylenterephtalamid) umfasst.

4. Schnittfester Stoff nach Anspruch 1, in Form eines Gestricks.

5. Artikel, der den schnittfesten Stoff nach Anspruch 1 umfasst.

6. Artikel nach Anspruch 5, in Form eines Handschuhs.

7. Verfahren zur Herstellung eines schnittfesten Stoffs, umfassend:
a) Mischen von
i) 20 bis 50 Gewichtsteilen einer Faser, ausgewählt aus der Gruppe der aliphatischen Polyamidfaser, der Polyolefinfaser, der Polyesterfaser, der Acrylfaser und Mischungen davon, und
ii) 50 bis 80 Gewichtsteilen einer Aramidfasermischung,
basierend auf 100 Gewichtsteilen der Fasern von i) und ii);
wobei die Aramidfasermischung mindestens eine erste Aramidfaser (5) mit einer linearen Dichte von 3,7 bis 6,7 dtex pro Filament und eine zweite Aramidfaser (6) mit einer linearen Dichte von 0,56 bis 5,0 dtex pro Filament umfasst; und
wobei der Unterschied in der linearen Dichte der Filamente zwischen der ersten Aramidfaser (5) und der zweiten Aramidfaser (6) 1,1 dtex pro Filament oder mehr beträgt;
b) Bilden eines Spinnstapelfasergarns aus dem Fasergemisch; und
c) Bilden eines Stoffs aus dem Spinnstapelfasergarn.

8. Verfahren nach Anspruch 7, wobei das Gemisch mindestens teilweise durch das Zusammenmischen der Fasern von i) und ii) und das Kardieren der Fasern durchgeführt wird, um ein Band zu bilden, das ein inneres Stapelfasergemisch enthält.

9. Verfahren nach Anspruch 7, wobei das Spinnstapelfasergarn unter Anwendung von Ringspinnen gebildet wird.

10. Verfahren nach Anspruch 7, wobei die erste und zweite Aramidfaser (5, 6) Poly(paraphenylenterephtalamid) umfasst.

11. Verfahren nach Anspruch 7, wobei der Stoff durch Stricken gebildet wird.

12. Verfahren nach Anspruch 11, wobei das Stricken durchgeführt wird, indem einer Strickmaschine ein Bündel Garne oder verzwirnte Garne gleichzeitig zugeführt werden, umfassend das Spinnstapelfasergarn aus dem Fasergemisch und ein oder mehrere andere Stapelfasergarne oder Endlosfilamentgarne.

13. Verfahren nach Anspruch 7, wobei der Stoff die Form eines Handschuhs hat.

## Revendications

1. Tissu résistant aux coupures, comprenant:
un fil comprenant un mélange intime de fibres discontinues, le mélange comprenant:
a) 20 à 50 parties en poids d'une fibre sélectionnées dans le groupe comprenant la fibre polyamide aliphatique, la fibre polyoléfine, la fibre polyester, la fibre acrylique et des mélanges de celles-ci; et
b) 50 à 80 parties en poids d'un mélange de fibre aramide,
sur la base de 100 parties en poids des fibres de a) et b);
le mélange de fibres aramides comprenant au moins une première fibre aramide (5) ayant une densité linéaire allant de 3,7 à 6,7 dtex par filament; et une deuxième fibre aramide (6) ayant une densité linéaire allant de 0,56 à 5,0 dtex par filamant; et
la différence de densité linéaire du filament entre la première fibre aramide (5) et la deuxième fibre aramide (6) est de 1,1 dtex par filament ou plus.

2. Tissu résistant aux coupures selon la revendication 1, dans lequel sur la base de 100 parties en poids des fibres de a) et b), la fibre de a) est présente en une quantité allant de 26 à 40 parties en poids et la fibre de b) est présente en une quantité allant de 60 à 70 parties en poids.

3. Tissu résistant aux coupures selon la revendication 1, dans lequel les première et deuxième fibres aramides (5, 6) comprennent du poly(paraphénylène téréphtalamide).

4. Tissu résistant aux coupres selon la revendication 1, sous la forme d'un tricotage.

5. Article comprenant le tissu résistant aux coupures selon la revendication 1.

6. Article selon la revendication 5, sous la forme d'un gant.

7. Procédé de fabrication d'un tissu résistant aux coupures, comprenant:
a) le mélange de:
i) 20 à 50 parties en poids d'une fibre sélectionnée dans le groupe comprenant la fibre polyamide aliphatique, la fibre polyoléfine, la fibre polyester, la fibre acrylique et des mélanges de celles-ci, et
ii) 50 à 80 parties en poids d'un mélange de fibre aramide,
sur la base de 100 parties en poids des fibres de i) et ii);
le mélange de fibre aramide comprenant au moins une première fibre aramide (5) ayant une densité linéaire allant de 3,7 à 6,7 dtex par filament; et une deuxième fibre aramide (6) ayant une densité linéaire allant de 0,56 à 5,0 dtex par filament; et
la différence de densité linéaire de filament entre la première fibre aramide (5) et la deuxième fibre aramide (6) étant de 1,1 dtex par filament ou plus;
b) la formation d'un fil filé de fibres discontinues à partir du mélange de fibres; et
c) la formation d'un tissu à partir du fil filé de fibres discontinues.

8. Procédé selon la revendication 7, dans lequel le mélange est accompli au moins en partie en mélangeant les fibres de i) et ii) et en cardant les fibres pour former une mèche contenant un mélange intime de fibres discontinues.

9. Procédé selon la revendication 7, dans lequel le fil filé de fibres discontinues est formé par filature à anneaux.

10. Procédé selon la revendication 7, dans lequel les première et deuxième fibres aramides (5, 6) comprennent du poly(paraphénylène téréphtalamide).

11. Procédé selon la revendication 7, dans lequel le tissu est formé par tricotage.

12. Procédé selon la revendication 11, dans lequel le tricotage est accompli en alimentant une machine à tricoter à la fois avec un faisceau de fils ou des fils retors comprenant le fil filé de fibres discontinues du mélange de fibres et un ou plusieurs autres fils de fibres discontinues ou des fils de filament continu.

13. Procédé selon la revendication 7, dans lequel le tissu est sous la forme d'un gant.
